



US010007199B2

(12) **United States Patent**  
Shimizu et al.

(10) **Patent No.:** US 10,007,199 B2  
(45) **Date of Patent:** Jun. 26, 2018

(54) **SINGLE-LAYER ELECTROPHOTOGRAPHIC PHOTOSENSITIVE MEMBER, PROCESS CARTRIDGE, AND IMAGE FORMING APPARATUS**

(71) Applicant: **KYOCERA Document Solutions Inc.**, Osaka (JP)

(72) Inventors: **Tomofumi Shimizu**, Osaka (JP); **Junichiro Otsubo**, Osaka (JP); **Yasuhiro Oishi**, Osaka (JP)

(73) Assignee: **KYOCERA Document Solutions Inc.**, Osaka (JP)

(\*) Notice: Subject to any disclaimer, the term of this patent is extended or adjusted under 35 U.S.C. 154(b) by 0 days. days.

(21) Appl. No.: **15/248,540**

(22) Filed: **Aug. 26, 2016**

(65) **Prior Publication Data**

US 2017/0068177 A1 Mar. 9, 2017

(30) **Foreign Application Priority Data**

Sep. 9, 2015 (JP) ..... 2015-177307

(51) **Int. Cl.**

**G03G 5/06** (2006.01)

**G03G 5/10** (2006.01)

**G03G 5/04** (2006.01)

**G03G 15/00** (2006.01)

**G03G 5/14** (2006.01)

(52) **U.S. Cl.**

CPC ..... **G03G 5/0607** (2013.01); **G03G 5/04**

(2013.01); **G03G 5/0609** (2013.01); **G03G**

**5/0631** (2013.01); **G03G 5/0696** (2013.01);

**G03G 5/102** (2013.01); **G03G 5/144**

(2013.01); **G03G 15/75** (2013.01); **G03G**

**2215/0129** (2013.01); **G03G 2215/0148**

(2013.01)

(58) **Field of Classification Search**

CPC ..... G03G 5/102; G03G 5/144; G03G 5/0607;

G03G 5/0609; G03G 5/0631; G03G 5/04;

G03G 5/0696

USPC ..... 430/69, 65, 78, 72

See application file for complete search history.

(56)

**References Cited**

U.S. PATENT DOCUMENTS

5,162,185 A \* 11/1992 Fukuda ..... G03G 5/144  
430/131  
5,430,526 A \* 7/1995 Ohkubo ..... G03G 15/0233  
399/159  
5,783,344 A \* 7/1998 Kobayashi ..... G03G 5/144  
430/65  
6,991,885 B2 \* 1/2006 Ojima ..... G03G 9/0819  
399/265  
2008/0305418 A1 \* 12/2008 Hamasaki ..... G03G 5/0564  
430/78  
2014/0242507 A1 \* 8/2014 Shimizu ..... G03G 5/0609  
430/56

FOREIGN PATENT DOCUMENTS

JP H04-278957 A 10/1992  
JP 2000-226354 \* 8/2000

OTHER PUBLICATIONS

Neufeldt, V. et al., Webster's New World Dictionary, Third College Edition, Simon & Schuster, Inc. NY (1988), p. 56.\*  
Japanese Patent Office JPlatPat machine-assisted English-language translation of JP 2000-226354 (pub. Aug. 2000).\*

\* cited by examiner

*Primary Examiner* — Janis L Dote

(74) *Attorney, Agent, or Firm* — Studebaker & Brackett PC

(57) **ABSTRACT**

A single-layer electrophotographic photosensitive member includes a conductive substrate and a photosensitive layer. The conductive substrate contains aluminum or an aluminum alloy. A surface of the conductive substrate has an aluminum oxide film or an aluminum alloy oxide film. The photosensitive layer is disposed directly on the conductive substrate. The photosensitive layer contains an electron transport material. The electron transport material has a reduction potential of at least -0.88 V and no greater than -0.66 V versus a reference electrode (Ag/Ag<sup>+</sup>). The single-layer electrophotographic photosensitive member has a leakage onset voltage of at least 5.0 kV in a high temperature and humidity environment at a temperature of 30° C. and a relative humidity of 80%. The leakage onset voltage is a voltage applied to the single-layer electrophotographic photosensitive member at which current leakage starts.

**8 Claims, 3 Drawing Sheets**



FIG. 1A



FIG. 1B



FIG. 2



FIG. 3

## 1

**SINGLE-LAYER ELECTROPHOTOGRAPHIC  
PHOTOSENSITIVE MEMBER, PROCESS  
CARTRIDGE, AND IMAGE FORMING  
APPARATUS**

INCORPORATION BY REFERENCE

The present application claims priority under 35 U.S.C. § 119 to Japanese Patent Application No. 2015-177307, filed on Sep. 9, 2015. The contents of this application are incorporated herein by reference in their entirety.

BACKGROUND

The present disclosure relates to a single-layer electro-photographic photosensitive member, a process cartridge, and an image forming apparatus.

An electrophotographic photosensitive member is used as an image bearing member in an electrophotographic image forming apparatus (for example, a printer or a multifunction peripheral). A generic electrophotographic photosensitive member includes a photosensitive layer. The photosensitive layer for example contains a charge generating material, a charge transport material (more specifically, a hole transport material or an electron transport material), and a resin (binder resin) for binding the aforementioned materials. The electrophotographic photosensitive member for example contains a charge generating material and a charge transport material in a single layer (photosensitive layer) and implements functions of charge generation and charge transport through the same layer. Such an electrophotographic photosensitive member is referred to as a single-layer electrophotographic photosensitive member. Alternatively, the photosensitive layer includes a charge generating layer containing a charge generating material and a charge transport layer containing a charge transport material. The electrophotographic photosensitive member including such a photosensitive layer is referred to as a multi-layer electrophotographic photosensitive member.

An electrophotographic photosensitive member described below is known. A multi-layer electrophotographic photosensitive member includes, as a photosensitive layer, a charge generating layer and a charge transport layer on a conductive substrate, and further includes a boehmite layer between the conductive substrate and the photosensitive layer.

SUMMARY

A single-layer electrophotographic photosensitive member according to an aspect of the present disclosure includes a conductive substrate and a photosensitive layer. The conductive substrate contains aluminum or an aluminum alloy. A surface of the conductive substrate has a film of an oxide of the aluminum or a film of an oxide of the aluminum alloy. The photosensitive layer is disposed directly on the conductive substrate. The photosensitive layer contains an electron transport material. The electron transport material has a reduction potential of at least -0.88 V and no greater than -0.66 V versus a reference electrode (Ag/Ag<sup>+</sup>). The single-layer electrophotographic photosensitive member according to the aspect of the present disclosure has a leakage onset voltage of at least 5.0 kV in a high temperature and humidity environment at a temperature of 30° C. and a relative humidity of 80%. The leakage onset voltage is a voltage applied to the single-layer electrophotographic photosensitive member at which current leakage starts.

## 2

A process cartridge according to another aspect of the present disclosure includes the above-described single-layer electrophotographic photosensitive member.

An image forming apparatus according to still another aspect of the present disclosure includes an image bearing member and a charger. The image bearing member is the above-described single-layer electrophotographic photosensitive member. The charger charges a surface of the image bearing member. The charger has a positive charging polarity.

BRIEF DESCRIPTION OF THE DRAWINGS

FIGS. 1A and 1B are schematic cross-sectional views each illustrating a structure of a single-layer electrophotographic photosensitive member according to a first embodiment of the present disclosure.

FIG. 2 is a schematic view illustrating a configuration of one form of an image forming apparatus according to a third embodiment of the present disclosure.

FIG. 3 is a schematic view illustrating a configuration of an alternative form of the image forming apparatus according to the third embodiment.

DETAILED DESCRIPTION

The following describes embodiments of the present disclosure in detail. However, the present disclosure is not in any sense limited by the following embodiments. The present disclosure can be implemented with appropriate alterations within the intended scope of the present disclosure. Note that although description is omitted as appropriate in some places in order to avoid repetition, such omission does not limit the essence of the present disclosure.

Hereinafter, the term “-based” may be appended to the name of a chemical compound in order to form a generic name encompassing both the chemical compound itself and derivatives thereof. Also, when the term “-based” is appended to the name of a chemical compound used in the name of a polymer, the term indicates that a repeating unit of the polymer originates from the chemical compound or a derivative thereof.

First Embodiment: Single-Layer  
Electrophotographic Photosensitive Member

The first embodiment of the present disclosure relates to a single-layer electrophotographic photosensitive member (hereinafter, may be referred to simply as a photosensitive member). The photosensitive member according to the first embodiment has excellent sensitivity and can reduce occurrence of black spots in a high temperature and humidity environment. The reason for the above is thought to be as follows.

First, for convenience, occurrence of black spots will be described. An electrophotographic image forming apparatus for example includes an image bearing member (photosensitive member), a charging section, a light exposure section, a development section, and a transfer section. The light exposure section forms an electrostatic latent image on a surface of the photosensitive member. The development section develops the electrostatic latent image into a toner image. In a situation in which the electrostatic latent image is not maintained on the surface of the photosensitive member after the light exposure performed by the light exposure section, a non-exposed region of the photosensitive member may go through development with toner during

the development performed by the development section. As a result, a plurality of dot images are formed on a non-image portion. Such an image defect may be referred to as black spots. Black spots are likely to occur particularly in a high temperature and humidity (for example, a temperature of 30° C. and a relative humidity of 80%) environment. The reason for the above is thought to be that moisture easily adheres to the surface of the photosensitive member in such a high temperature and humidity environment.

The photosensitive member according to the first embodiment has an oxide film as a surface of the conductive substrate. The photosensitive layer contains an electron transport material. A reduction potential of the electron transport material is at least -0.88 V and no greater than -0.66 V versus a reference electrode (Ag/Ag<sup>+</sup>). A leakage onset voltage of the photosensitive member according to the first embodiment is at least 5.0 kV in a high temperature and humidity (for example, a temperature of 30° C. and a relative humidity of 80%) environment. The photosensitive member as described above tends to inhibit hole injection into the photosensitive layer. It is thought that an electrostatic latent image formed on the surface of the photosensitive member is therefore maintained in a stable manner. Thus, the photosensitive member according to the first embodiment can reduce occurrence of black spots even in a high temperature and humidity environment.

Furthermore, since the reduction potential of the electron transport material is at least -0.88 V and no greater than -0.66 V versus the reference electrode (Ag/Ag<sup>+</sup>), the lowest unoccupied molecular orbital (LUMO) of the electron transport material is in the vicinity of the LUMO of the charge generating material. Accordingly, the electron transport material receives electrons from the charge generating material more readily. The photosensitive member according to the first embodiment therefore has excellent sensitivity.

The leakage onset voltage refers to a voltage applied to the photosensitive member at which current leakage starts. The leakage onset voltage is measured as a lowest value of the voltage applied to the photosensitive member at which dielectric breakdown occurs while the voltage is being increased. The leakage onset voltage can be measured using a pressure-resistant tester (testing instrument fabricated by KYOCERA Document Solutions Inc.). A method for measuring the leakage onset voltage will be described later in detail in Examples. Preferably, the leakage onset voltage in a high temperature and humidity environment is at least 5.0 kV and no greater than 9.0 kV.

The following describes the photosensitive member with reference to FIGS. 1A and 1B. FIGS. 1A and 1B are schematic cross-sectional views each illustrating a structure of a photosensitive member 1. The photosensitive member 1 includes a conductive substrate 2 and a photosensitive layer 3. The photosensitive layer 3 is disposed directly on the conductive substrate 2. For example, the photosensitive layer 3 may be disposed directly on the conductive substrate 2 as illustrated in FIG. 1A. The photosensitive layer 3 may be exposed as an outermost layer as illustrated in FIG. 1A. A protective layer 5 may be disposed on the photosensitive layer 3 as illustrated in FIG. 1B. The following describes the conductive substrate and the photosensitive layer.

#### [1. Conductive Substrate]

The conductive substrate 2 contains aluminum or an aluminum alloy. As a result of the conductive substrate 2 containing aluminum or an aluminum alloy, charge transfer from the photosensitive layer 3 to the conductive substrate 2 tends to be improved. The aluminum alloy is an alloy of aluminum with elements other than aluminum. Examples of elements other than aluminum include manganese (Mn), silicon (Si), magnesium (Mg), copper (Cu), iron (Fe), chromium (Cr), titanium (Ti), and zinc (Zn). An aluminum alloy

may contain one of the elements listed above as an element other than aluminum or may contain two or more of the elements listed above. Examples of aluminum alloys that can be used include Al—Mn alloys (1153000 series), Al—Mg alloys (JIS5000 series), and Al—Mg—Si alloys (JIS6000 series).

The conductive substrate 2 has an aluminum oxide film or an aluminum alloy oxide film as a surface thereof. The aluminum oxide film or the aluminum alloy oxide film is for example formed by performing an oxidation treatment on the surface of the conductive substrate 2.

Preferably, a proportion R of oxygen atoms present in the aluminum oxide film or the aluminum alloy oxide film is at least 20% and no greater than 50%. The proportion R of oxygen atoms can be determined in accordance with equation (1).

$$R = [A_O / (A_O + A_{Al})] \times 100 \quad \text{Equation (1)}$$

In the equation (1),  $A_O$  represents an oxygen atom concentration, which is determined by measuring the aluminum oxide film or the aluminum alloy oxide film by energy dispersive X-ray spectroscopy (EDX).  $A_{Al}$  represents an aluminum atom concentration, which is determined by measuring the aluminum oxide film or the aluminum alloy oxide film by energy dispersive X-ray spectroscopy.

The oxygen atom concentration and the aluminum atom concentration can be measured using an energy dispersive X-ray spectrometer ("JSM-6380LV", product of JEOL Ltd.). A method for measuring the oxygen atom concentration and the aluminum atom concentration will be described later in detail in the Examples.

As a result of the proportion R of oxygen atoms being at least 20%, the oxide film of the conductive substrate 2 has a suitable electric resistance. Accordingly, charge injection (electron injection) from the conductive substrate 2 to the photosensitive layer 3 can be restricted. As a result of the proportion R of oxygen atoms being no greater than 50%, inhibition of hole transport from the photosensitive layer 3 to the conductive substrate 2 is difficult.

Preferably, the aluminum oxide film or the aluminum alloy oxide film has a thickness of at least 0.15 μm and no greater than 0.35 μm. As a result of having a thickness of at least 0.15 μm and no greater than 0.35 μm, the oxide film of the conductive substrate 2 has a suitable electric resistance. Consequently, charge injection (electron injection) from the conductive substrate 2 to the photosensitive layer can be restricted. Furthermore, hole transport from the photosensitive layer 3 to the conductive substrate 2 is less likely to be inhibited. The thickness of the oxide film can for example be measured using a reflective/transmissive thin film thickness measuring device ("NANOCALC-VIS", product of Tokyo Instruments, Inc.). A method for measuring the thickness of the oxide film will be described later in detail in the Examples.

The shape of the conductive substrate 2 may be selected as appropriate to match the structure of an image forming apparatus in which the conductive substrate 2 is to be used. The conductive substrate 2 may for example be sheet-shaped or drum-shaped. The thickness of the conductive substrate 2 can be selected as appropriate according to the shape of the conductive substrate 2.

#### [2. Photosensitive Layer]

As mentioned above, the photosensitive layer 3 contains an electron transport material. The photosensitive layer 3 may contain a charge generating material, a hole transport material, and various additives as necessary. The following describes the charge generating material, the electron transport material, the hole transport material, the binder resin, and additives.

## (2-1. Charge Generating Material)

No particular limitations are placed on the charge generating material other than being a charge generating material that can be used in photosensitive members. Examples of charge generating materials that can be used include phthalocyanine-based pigments, perylene pigments, bisazo pigments, dithioketopyrrolopyrrole pigments, metal-free naphthalocyanine pigments, metal naphthalocyanine pigments, squaraine pigments, tris-azo pigments, indigo pigments, azulenium pigments, cyanine pigments, powders of inorganic photoconductive materials (for example, selenium, selenium-tellurium, selenium-arsenic, cadmium sulfide, or amorphous silicon), pyrylium salts, anthranthrone-based pigments, triphenylmethane-based pigments, threne-based pigments, toluidine-based pigments, pyrazoline-based pigments, and quinacridone-based pigments.

Examples of phthalocyanine-based pigments that can be used include metal-free phthalocyanine represented by chemical formula (CGM-1) and metal phthalocyanine. Examples of metal phthalocyanine that can be used include titanyl phthalocyanine represented by chemical formula (CGM-2) and phthalocyanine having a metal other than titanium oxide as a coordination center (specific examples include V-form hydroxygallium phthalocyanine). The phthalocyanine-based pigment may be crystalline or non-crystalline. No particular limitations are placed on the crystal structure (for example,  $\alpha$ -form,  $\beta$ -form, or Y-form) of the phthalocyanine-based pigments, and phthalocyanine-based pigments having various different crystal structures may be used.

(CGM-1)



(CGM-2)



Examples of crystalline metal-free phthalocyanine that can be used include metal-free phthalocyanine having an

X-form crystal structure (hereinafter, may be referred to as X-form metal-free phthalocyanine). Examples of crystalline titanyl phthalocyanine include titanyl phthalocyanine having an  $\alpha$ -form,  $\beta$ -form, or Y-form crystal structure.

A single charge generating material having an absorption wavelength in a desired region or a combination of two or more charge generating materials may be used. Also, for example in a digital optical system image forming apparatus, the photosensitive member 1 that is sensitive to a range of wavelengths that are greater than or equal to 700 nm is preferably used. Accordingly, for example, a phthalocyanine-based pigment is preferable, and metal-free phthalocyanine or titanyl phthalocyanine is more preferable. One charge generating material may be used independently, or two or more charge generating materials may be used in combination. The digital optical system image forming apparatus may for example be a laser beam printer or facsimile machine in which a light source such as a semiconductor laser is used.

An anthranthrone-based pigment or a perylene-based pigment is favorably used as a charge generating material in the photosensitive member 1 that is applied to an image forming apparatus including a short-wavelength laser light source. The short-wavelength laser light for example has a wavelength of at least 350 nm and no greater than 550 nm.

The charge generating material is preferably contained in an amount of at least 0.1 parts by mass and no greater than 50 parts by mass relative to 100 parts by mass of the binder resin, and more preferably at least 0.5 parts by mass and no greater than 30 parts by mass.

## (2-2. Electron Transport Material)

A reduction potential of the electron transport material is at least  $-0.88$  V and no greater than  $-0.66$  V versus a reference electrode (Ag/Ag<sup>+</sup>). As a result of the reduction potential of the electron transport material being at least  $-0.88$  V and no greater than  $-0.66$  V, the photosensitive member has excellent sensitivity and can reduce occurrence of black spots in a high temperature and humidity environment. A method for measuring the reduction potential of the electron transport material will be described later in the Examples.

Preferably, the electron transport material is a compound represented by general formula (1), general formula (2), or general formula (3).

(1)



(2)



7

-continued



(3)

8

(ETM-1)



10

(ETM-2)



15

(ETM-3)



20

25

30

35

40

45

50

55

60

65

In the general formulae (1), (2), and (3), R<sup>1</sup>, R<sup>2</sup>, R<sup>3</sup>, R<sup>4</sup>, R<sup>5</sup>, R<sup>6</sup>, R<sup>7</sup>, and R<sup>8</sup> each represent, independently of one another, an alkyl group that may have a substituent selected from the group consisting of alkoxy groups and halogen atoms or an aryl group that may have a substituent selected from the group consisting of alkoxy groups and halogen atoms.

The alkyl group represented by each of R<sup>1</sup> to R<sup>8</sup> in the general formulae (1) to (3) is preferably an alkyl group having a carbon number of at least 1 and no greater than 5. Examples of alkyl groups each having a carbon number of at least 1 and no greater than 5 include a methyl group, an ethyl group, an n-propyl group, an isopropyl group, an n-butyl group, a sec-butyl group, a tert-butyl group, an pentyl group, and a tert-pentyl group. Of the alkyl groups listed above, an isopropyl group, a tert-butyl group, or a tert-pentyl group is more preferable.

The alkyl group represented by each of R<sup>1</sup> to R<sup>8</sup> in the general formulae (1) to (3) may have an alkoxy group or a halogen atom as a substituent. Preferably, the alkoxy group is for example an alkoxy group having a carbon number of at least 1 and no greater than 5. Examples of alkoxy groups each having a carbon number of at least 1 and no greater than 5 include a methoxy group, an ethoxy group, an n-propoxy group, an isopropoxy group, an n-butoxy group, a sec-butoxy group, a tert-butoxy group, an n-pentoxy group, and a tert-pentoxy group. Examples of halogen atoms include a fluorine atom, a chlorine atom, a bromine atom, and an iodine atom.

The aryl group represented by each of R<sup>1</sup> to R<sup>8</sup> in the general formulae (1) to (3) is preferably an aryl group having a carbon number of at least 6 and no greater than 10, and more preferably a phenyl group or a naphthyl group. The aryl group represented by each of R<sup>1</sup> to R<sup>8</sup> in the general formulae (1) to (3) may have an alkoxy group or a halogen atom as a substituent. The substituent of the aryl group represented by each of R<sup>1</sup> to R<sup>8</sup> in the general formulae (1) to (3) is a substituent selected from the group consisting of alkoxy groups and halogen atoms. The alkoxy group that may be a substituent of the aryl group is as defined for the alkoxy groups that may be a substituent of the alkyl group represented by each of R<sup>1</sup> to R<sup>8</sup> in the general formulae (1) to (3). The halogen atom that may be a substituent of the aryl group is as defined for the halogen atom that may be a substituent of the alkyl group represented by each of R<sup>1</sup> to R<sup>8</sup> in the general formulae (1) to (3). The halogen atom is preferably a chlorine atom.

Preferably, R<sup>1</sup> to R<sup>4</sup> and R<sup>6</sup> to R<sup>8</sup> in the general formulae (1), (2), and (3) each represent, independently of one another, an alkyl group having a carbon number of at least 1 and no greater than 5. In the general formula (2), R<sup>6</sup> preferably represents a phenyl group having a halogen atom, and more preferably a dichlorophenyl group.

Specific examples of electron transport materials that can be used include compounds represented by chemical formulae (ETM-1) to (ETM-3) (hereinafter, may be referred to as compounds (ETM-1) to (ETM-3)).

The electron transport material may contain an optional electron transport material in addition to the electron transport material having a reduction potential such as described above. No particular limitations are placed on the optional electron transport material other than being applicable to the photosensitive member 1. Examples of electron transport materials that can be used include quinone-based compounds, diimide-based compounds, hydrazone-based compounds, malononitrile-based compounds, thiopyran-based compounds, trinitrothioxanthone-based compounds, 3,4,5,7-tetranitro-9-fluorenone-based compounds, dinitroanthracene-based compounds, dinitroacridine-based compounds, tetracyanoethylene, 2,4,8-trinitrothioxanthone, dinitrobenzene, dinitroacridine, succinic anhydride, maleic anhydride, and dibromomaleic anhydride. Examples of quinone-based compounds that can be used include diphenoquinone-based compounds, azoquinone-based compounds, anthraquinone-based compounds, naphthoquinone-based compounds, and dinitroanthraquinone-based compounds. Any one of the electron transport materials listed above may be used independently, or any two or more of the electron transport materials listed above may be used in combination.

The electron transport material is preferably contained in an amount of at least 5 parts by mass and no greater than 100

parts by mass relative to 100 parts by mass of the binder resin, and more preferably at least 10 parts by mass and no greater than 80 parts by mass.

(2-3. Hole Transport Material)

No particular limitations are placed on the hole transport material other than being applicable to the photosensitive member 1. A nitrogen containing cyclic compound or a condensed polycyclic compound may for example used as the hole transport material. Examples of nitrogen-containing cyclic compounds and condensed polycyclic compounds that can be used include triphenylamine derivatives, diamine derivatives (specific examples include N,N,N',N'-tetraphenylbenzidine derivatives, N,N,N',N'-tetraphenylphenylenediamine derivatives, di(aminophenylethenyl)benzene derivatives, and N,N,N',N'-tetraphenylphenanthrylenediamine derivatives), oxadiazole-based compounds (specific examples include 2,5-di(4-methylaminophenyl)-1,3,4-ox-

adiazole), styryl-based compounds (specific example include 9-(4-diethylaminostyryl)anthracene), carbazole-based compounds (specific examples include polyvinyl carbazole), organic polysilane compounds, pyrazoline-based compound (specific examples include 1-phenyl-3-(p-dimethylaminophenyl)pyrazoline), hydrazone-based compounds, indole-based compounds, oxazole-based compounds, isoxazole-based compounds, thiazole-based compounds, thiadiazole-based compounds, imidazole-based compounds, pyrazole-based compounds, and triazole-based compounds. Any one of the hole transport materials listed above may be used independently, or any two or more of the hole transport materials listed above may be used in combination.

15 Specific examples of hole transport materials that can be used include compounds represented by chemical formulae (HTM-1) to (HTM-6) (hereinafter, may be referred to as compounds (HTM-1) to (HTM-6)).



11



12

-continued  
(HTM-5)

(HTM-6)



20 The hole transport material is preferably contained in an amount of at least 10 parts by mass and no greater than 200 parts by mass relative to 100 parts by mass of the binder resin, and more preferably at least 10 parts by mass and no greater than 100 parts by mass.

(2-4. Binder Resin)

The photosensitive layer **3** can contain a binder resin. Examples of binder resins that can be used include thermoplastic resins, thermosetting resins, and photocurable resins. Examples of thermoplastic resins that can be used include polyester resins, polycarbonate resins, styrene-based resins, styrene-butadiene resins, styrene-acrylonitrile copolymers, styrene-maleic acid copolymers, styrene-acrylic acid copolymers, acrylic copolymers, polyethylene resins, ethylene-vinyl acetate copolymers, chlorinated polyethylene resins, polyvinyl chloride resins, polypropylene resins, ionomers, vinyl chloride-vinyl acetate copolymers, alkyd resins, polyamide resins, urethane resins, polyarylate resins, polysulfone resins, diallyl phthalate resins, ketone resins, polyvinyl butyral resins, and polyether resins. Examples of thermosetting resins that can be used include silicone resins, epoxy resins, phenolic resins, urea resins, melamine resins, and

25 other crosslinkable thermosetting resins. Examples of photocurable resins that can be used include epoxy acrylate resins and urethane-acrylate copolymers. Any one of the resins listed above may be used independently, or any two or more of the resins listed above may be used in combination.

30 Of the binder resins listed above, a polycarbonate resin is preferable. As a result of the binder resin being a polycarbonate resin, the photosensitive layer **3** having excellent balance in terms of processability, mechanical properties, 35 optical properties, and abrasion resistance is readily obtained. In terms of readily improving toner image transferability of the photosensitive member **1**, the polycarbonate resin is preferably a bisphenol Z polycarbonate resin, a bisphenol CZ polycarbonate resin, or a bisphenol C polycarbonate resin, and more preferably a resin represented by chemical formula (Z), chemical formula (C), or chemical formula (CZ) shown below. The number attached to each 40 repeating unit in the chemical formulae (Z), (C), and (CZ) indicates the molar ratio of the repeating unit relative to the total number of moles of repeating units included in the corresponding resin.

(Z)



(C)



(CZ)



The binder resin preferably has a viscosity average molecular weight of at least 40,000, and more preferably at least 40,000 and no greater than 52,500. As a result of the binder resin having a viscosity average molecular weight of at least 40,000, abrasion resistance of the photosensitive member 1 can be readily improved. As a result of the binder resin having a viscosity average molecular weight of no greater than 52,500, the binder resin has a high tendency to dissolve in a solvent and viscosity of an application liquid for formation of the photosensitive layer 3 has a low tendency to be too high when the photosensitive layer 3 is formed. Consequently, the photosensitive layer 3 can be readily formed.

(2-5. Additives)

Examples of additives that can be used include antioxidants (specific examples include antioxidants, radical scavengers, singlet quenchers, and ultraviolet absorbing agents), softeners, surface modifiers, extending agents, thickeners, dispersion stabilizers, waxes, acceptors, donors, surfactants, plasticizers, sensitizers, and leveling agents. Examples of antioxidants include hindered phenols, hindered amines, paraphenylenediamine, arylalkanes, hydroquinone, spirochromanes, spiroindanones, derivatives of any of the above compounds, organosulfur compounds, and organophosphorus compounds.

Through the above, the photosensitive member 1 according to the first embodiment has been described with reference to FIGS. 1A and 1B. The photosensitive member 1 according to the first embodiment has excellent sensitivity and can reduce occurrence of black spots in a high temperature and humidity environment.

Second Embodiment: Photosensitive Member Production Method

The following describes a production method of the photosensitive member 1 with reference to FIGS. 1A and 1B. The production method of the photosensitive member 1 includes an oxide film formation step and a photosensitive layer formation step. The following describes the oxide film formation step and the photosensitive layer formation step.

[1. Oxide Film Formation Step]

In the oxide film formation step, a conductive substrate is immersed in water, taken out of water, and heated to form an aluminum oxide film or an aluminum alloy oxide film on a surface of the conductive substrate. The water has a volume resistivity of at least  $1.0 \times 10^6 \Omega \cdot \text{cm}$ . The water has a temperature of at least 70° C. and less than 80° C. The conductive substrate is immersed in water for at least 60 seconds and no greater than 90 seconds. The conductive substrate may be heated at ambient atmosphere. The heating temperature is at least 110° C. and no greater than 150° C., and more preferably at least 120° C. and no greater than 140° C. The heating time may be at least 5 minutes and no greater than 30 minutes.

The oxide film formation step may further include an ionized alkaline water immersion step. In the ionized alkaline water immersion step, the conductive substrate 2 is immersed in ionized alkaline water prior to formation of the oxide film. Through the above, at least a portion of an oxide film already formed on the surface of the conductive substrate 2 can be removed. As a result, a new oxide film can be formed on the conductive substrate 2, and the conductive substrate 2 having a desired electric resistance can be readily formed.

Preferably, the ionized alkaline water has a pH of at least 9 and no greater than 12. Preferably, the conductive substrate

2 is immersed in the ionized alkaline water for at least 20 seconds and no greater than 120 seconds.

Subsequently, the conductive substrate is taken out of the ionized alkaline water and water adhering thereto is removed. The water may be removed by heating. The heating may be performed at a heating temperature of at least 110° C. and no greater than 150° C. at ambient atmosphere. The heating time may be at least 5 minutes and no greater than 30 minutes. The conductive substrate 2 may for example be heated using an oven.

[2. Photosensitive Layer Formation Step]

In the photosensitive layer formation step, an application liquid for photosensitive layer formation (hereinafter, may be referred to simply as an application liquid) is applied onto the conductive substrate 2, and at least a portion of a solvent contained in the applied application liquid is removed to form the photosensitive layer 3. The application liquid contains at least an electron transport material and a solvent. The photosensitive layer formation step for example includes an application liquid preparation step, an application step, and a drying step. The following describes the application liquid preparation step, the application step, and the drying step.

(2-1. Application Liquid Preparation Step)

In the application liquid preparation step, the application liquid is prepared. The application liquid may contain a charge generating material, a hole transport material, a binder resin, or an additive as necessary. The application liquid can for example be prepared by dissolving or dispersing the electron transport material represented by the general formula (1), (2), or (3) and an optional component (specific examples include a charge generating material, a hole transport material, a binder resin, and an additive) in the solvent.

No particular limitations are placed on the solvent contained in the application liquid other than that the components of the application liquid is soluble or dispersible in the solvent. Examples of solvents that can be used include alcohols (specific examples include methanol, ethanol, isopropanol, and butanol), aliphatic hydrocarbons (specific examples include n-hexane, octane, and cyclohexane), aromatic hydrocarbons (specific examples include benzene, toluene, and xylene), halogenated hydrocarbons (specific examples include dichloromethane, dichloroethane, carbon tetrachloride, and chlorobenzene), ethers (specific examples include dimethyl ether, diethyl ether, tetrahydrofuran, ethylene glycol dimethyl ether, and diethylene glycol dimethyl ether), ketones (specific examples include acetone, methyl ethyl ketone, and cyclohexanone), esters (specific examples include ethyl acetate and methyl acetate), dimethyl formaldehyde, N,N-dimethylformamide (DMF), and dimethyl sulfoxide. One of the solvents listed above may be used independently, or two or more of the solvents listed above may be used in combination. Of the solvents listed above, a non-halogenated solvent is preferable.

The application liquid is prepared by mixing the components in order to cause dissolution or dispersion in the solvent. Mixing, dissolving, or dispersing can for example be performed using a bead mill, a roll mill, a ball mill, an attritor, a paint shaker, or an ultrasonic disperser.

The application liquid may for example contain a surfactant or a leveling agent in order to improve dispersibility of the components or improve surface flatness of the photosensitive layer 3 to be formed.

(2-2. Application Step)

In the application step, the application liquid is applied onto the conductive substrate 2. No particular limitations are placed on the method by which the application liquid is

applied so long as the method for example enables uniform application of the application liquid onto the conductive substrate **2**. Examples of the application method include dip coating, spray coating, spin coating, and bar coating.

Preferably, the application liquid is applied by dip coating in terms of readily adjusting the thickness of the photosensitive layer **3** to a desired value. In the application step that is performed by dip coating, the conductive substrate **2** is immersed in the application liquid. Subsequently, the conductive substrate **2** is drawn out of the application liquid. Through the above, the application liquid is applied onto the conductive substrate **2**.

(2-3. Drying Step)

In the drying step, at least a portion of the solvent contained in the application liquid applied to the conductive substrate **2** is removed. No specific limitations are placed on the method by which the solvent in the application liquid is removed other than being a method that enables removal (specific examples include evaporation) of at least a portion of the solvent in the application liquid. Examples of methods that can be used to remove the solvent include heating, pressure reduction, and a combination of heating and pressure reduction. Specific examples thereof include heat treatment (hot-air drying) using a high-temperature dryer or a reduced pressure dryer. The heat treatment is for example performed for at least 3 minutes and no greater than 120 minutes at a temperature of at least 40° C. and no greater than 150° C.

The production method of the photosensitive member **1** may further include a step of forming the protective layer **5** as necessary. A known method is selected as appropriate for the step of forming the protective layer **5**.

Through the above, the production method of the photosensitive member **1** according to the second embodiment has been described with reference to FIGS. 1A and 1B. The production method of the photosensitive member **1** according to the second embodiment can produce a photosensitive member that has excellent sensitivity and that can reduce occurrence of black spots in a high temperature and humidity environment.

Third Embodiment: Image Forming Apparatus

The third embodiment of the present disclosure relates to an image forming apparatus. The image forming apparatus includes the photosensitive member **1** as an image bearing member. The photosensitive member **1** has excellent sensitivity and can reduce occurrence of black spots in a high temperature and humidity environment as mentioned for the first embodiment. The image forming apparatus including such a photosensitive member **1** is therefore thought to be capable of forming images while reducing occurrence of black spots in a high temperature and humidity environment with the photosensitive member **1** having excellent sensitivity.

The following describes the image forming apparatus according to the third embodiment with reference to FIGS. 2 and 3. First, description is given of an example in which the image forming apparatus adopts an intermediate transfer process with reference to FIG. 2. FIG. 2 is a schematic view illustrating a configuration of one form of the image forming apparatus according to the third embodiment. An image forming apparatus **6** includes the photosensitive member **1** according to the first embodiment as an image bearing member.

The image forming apparatus **6** according to the third embodiment includes the image bearing member **1** and a

charging section **27**, which is equivalent to a charger. The charging section **27** charges the surface of the image bearing member **1**. The charging section **27** has a positive charging polarity. The image forming apparatus **6** according to the third embodiment further includes a light exposure section **28**, which is equivalent to a light exposure device, a development section **29**, and a transfer section **26**. The light exposure section **28** exposes the charged surface of the image bearing member **1** to light to form an electrostatic latent image on the surface of the image bearing member **1**. The development section **29** develops the electrostatic latent image into a toner image. The transfer section **26** transfers the toner image from the image bearing member **1** to a transfer target **38**. In a configuration in which the image forming apparatus **6** adopts the intermediate transfer process, as illustrated in FIG. 2, the transfer section **26** is equivalent to primary transfer rollers **33**. The transfer target **38** is equivalent to an intermediate transfer member (for example, an intermediate transfer belt **20**).

No particular limitations are placed on the image forming apparatus **6** other than being an electrophotographic image forming apparatus. The image forming apparatus **6** may for example be a monochrome image forming apparatus or a color image forming apparatus. In order to form toner images of different colors using toners of different colors, the image forming apparatus **6** may be a tandem color image forming apparatus.

The following describes the image forming apparatus **6** taking a tandem color image forming apparatus as an example. The image forming apparatus **6** includes a plurality of the image bearing members **1** arranged side-by-side in a specific direction and a plurality of the development sections **29**. The development sections **29** are disposed opposite to the image bearing members **1** in one-to-one correspondence. The development sections **29** each include a development roller. Each development roller conveys and supplies a toner to the surface of a corresponding one of the image bearing members **1** by bearing the toner thereon.

As illustrated in FIG. 2, the image forming apparatus **6** further includes a boxlike apparatus housing **7**. A paper feed section **8**, an image forming section **9**, and a fixing section **10** are disposed inside the apparatus housing **7**. The paper feed section **8** feeds paper **P**. The image forming section **9** transfers toner images based on image data to the paper **P** while conveying the paper **P** fed by the paper feed section **8**. After an unfixed toner image is transferred onto the paper **P** by the image forming section **9**, the fixing section **10** fixes the unfixed toner image to the paper **P**. Furthermore, a paper ejection section **11** is provided in a top surface of the apparatus housing **7**. After the unfixed toner image is fixed to the paper **P** by the fixing section **10**, the paper ejection section **11** ejects the paper **P**.

The paper feed section **8** includes a paper feed cassette **12**, a first pickup roller **13**, a plurality of paper feed rollers **14**, and a pair of registration rollers **17**. The paper feed cassette **12** is attachable to and detachable from the apparatus housing **7**. Various sizes of paper **P** can be loaded into the paper feed cassette **12**. The first pickup roller **13** is located above a left side of the paper feed cassette **12**. The first pickup roller **13** picks up paper **P** stored in the paper feed cassette **12** one sheet at a time. The paper feed rollers **14** convey the paper **P** picked up by the first pickup roller **13**. The pair of registration rollers **17** temporarily halts the paper **P** conveyed by the paper feed rollers **14** and subsequently supplies the paper **P** to the image forming section **9** at a specific timing.

The paper feed section 8 may further include a manual feed tray (not illustrated) and a second pickup roller 18. The manual feed tray is attached to a left side surface of the apparatus housing 7. The second pickup roller 18 picks up paper P loaded on the manual feed tray. The paper P picked up by the second pickup roller 18 is conveyed by the paper feed rollers 14 and is supplied to the image forming section 9 at a specific timing by the pair of registration rollers 17.

The image forming section 9 includes an image forming unit 19, the intermediate transfer belt 20, and a secondary transfer roller 21. The image forming unit 19 performs primary transfer of a toner image onto a circumferential surface of the intermediate transfer belt 20 (contact surface with the image bearing members 1). The toner image that undergoes primary transfer is formed based on image data transmitted from a higher-level device, such as a computer. The secondary transfer roller 21 performs secondary transfer of the toner image on the intermediate transfer belt 20 to the paper P fed from the paper feed cassette 12.

The image forming unit 19 includes a yellow toner supply unit 25, a magenta toner supply unit 24, a cyan toner supply unit 23, and a black toner supply unit 22. In the image forming unit 19, the yellow toner supply unit 25, the magenta toner supply unit 24, the cyan toner supply unit 23, and the black toner supply unit 22 are arranged in order from upstream (right side in FIG. 2) to downstream in a circulation direction of the intermediate transfer belt 20 relative to the yellow toner supply unit 25 as a reference point. The image bearing member 1 is located at a central position in each of the units 22, 23, 24, and 25. The image bearing members 1 are provided such as to be rotatable in an arrow direction (clockwise). Note that each of the units 22, 23, 24, and 25 may be a process cartridge described below that is attachable to and detachable from a main body of the image forming apparatus 6.

Each charging section 27, each light exposure section 28, and each development section 29 are located around a corresponding one of the image bearing members 1 in order from upstream in a rotation direction of the image bearing member 1 relative to the charging section 27 as a reference point.

A static eliminator (not illustrated) and a cleaning device (not illustrated) may be provided upstream of the charging section 27 in the rotation direction of the image bearing member 1. The static eliminator eliminates static from a circumferential surface (surface) of the image bearing member 1 after primary transfer of the toner image onto the intermediate transfer belt 20 has been performed. After the surface of the image bearing member 1 has been subjected to cleaning and static elimination by the cleaning device and the static eliminator, the surface is subjected to a new charging process as the circumferential surface passes the charging section 27. In a configuration in which the image forming apparatus 6 includes cleaning devices and static eliminators, each charging section 27, each light exposure section 28, each development section 29, each cleaning device, and each static eliminator are provided around a corresponding one of the image bearing members 1 in order from upstream in the rotation direction of the image bearing member 1. The development section 29 may function as a cleaning device. The development section 29 will be described later in detail.

As already mentioned above, the charging section 27 charges the surface of the image bearing member 1. More specifically, the charging section 27 uniformly charges the surface of the image bearing member 1. No specific limitations are placed on the charging section 27 other than

enabling uniform charging of the circumferential surface of the image bearing member 1. The charging section 27 may be a non-contact charging section or a contact charging section. The non-contact charging section 27 applies voltage to the image bearing member 1 without being in contact with the image bearing member 1. When the charging section 27 is a non-contact charging section, the charging section 27 is for example a corona discharge charging section and, more specifically, is for example a corotron charging device or a scorotron charging device. The contact charging section applies voltage to the image bearing member 1 while in contact with the image bearing member 1. When the charging section 27 is a contact charging section, the charging section 27 is for example a charging roller or a charging brush. Discharge of active gases (for example, ozone and nitrogen oxides) generated by the charging section 27 can be inhibited by using a contact charging section as the charging section 27. As a result, deterioration of the photosensitive layer 3 due to active gases can be inhibited while also achieving a design that takes into consideration use in an office environment.

The charging section 27 can charge the surface of the image bearing member 1 while in contact with the image bearing member 1 as described above. That is, the image forming apparatus 6 according to the third embodiment can adopt a so-called contact charging process. In the image forming apparatus 6 that adopts the contact charging process, typically, each charging section 27 and the corresponding image bearing member 1 are in contact with one another during development, and therefore a toner-component matter, or a non-toner-component matter is likely to remain on and adhere to the surface of the image bearing member 1. It is thought that the matter adhering to the surface of the image bearing member 1 absorbs moisture and prevents an electrostatic latent image formed on the surface of the image bearing member 1 from being maintained in a stable manner. As described above, the image forming apparatus 6 according to the third embodiment restricts hole injection to the photosensitive layers and therefore can reduce occurrence of black spots in a high temperature and humidity environment. The image forming apparatus 6 according to the third embodiment can therefore form images while reducing occurrence of black spots in a high temperature and humidity environment even through the contact charging process. Hereinafter, a toner-component matter or a non-toner-component matter remaining on the surface of the image bearing member 1 may be referred to as a residual matter. The toner-component matter is for example a toner or an external additive detached from the toner. The non-toner-component matter is for example paper dust.

The charging roller is for example a charging roller that passively rotates in accordance with rotation of the image bearing member 1 while in contact with the surface of the image bearing member 1. Furthermore, the charging roller is for example a charging roller for which at least a surface part thereof is made from a resin. In a more specific example, the charging roller is a charging roller that includes a metal core that is rotatably supported, a resin layer formed on the metal core, and a voltage applying section that applies voltage to the metal core. In a configuration in which the charging section 27 includes a charging roller such as described above, the charging section 27 can charge the surface of the image bearing member 1, which is in contact therewith via the resin layer, through the voltage applying section applying voltage to the metal core.

No specific limitations are placed on the resin used to make the resin layer of the charging roller other than

enabling favorable charging of the surface of the image bearing member 1. Specific examples of the resin used to make the resin layer include silicone resins, urethane resins, and silicone modified resins. The resin layer may contain an inorganic filler.

No specific limitations are placed on the voltage applied by the charging section 27. The voltage applied by the charging section 27 is for example an alternating current voltage, a composite voltage of an alternating current voltage superimposed on a direct current voltage, or a direct current voltage. Preferably, the charging section 27 only applies a direct current voltage. The charging section 27 that only applies a direct current voltage is advantageous as described below compared to the charging section 27 that applies an alternating current voltage or to the charging section 27 that applies a superimposed voltage. In a configuration in which the charging section 27 only applies a direct current voltage, the value of voltage applied to the image bearing member 1 is constant, and therefore it is easy to uniformly charge the surface of the image bearing member 1 to a specified potential. Furthermore, in a configuration in which the charging section 27 only applies a direct current voltage, the amount of abrasion of the photosensitive layer 3 tends to be smaller. It is thought that as a result, suitable images can be formed. The direct current voltage applied to the image bearing member 1 by the charging section 27 is preferably at least 1,000 V and no greater than 2,000 V, more preferably at least 1,200 V and no greater than 1,800 V, and particularly preferably at least 1,400 V and no greater than 1,600 V.

The light exposure section 28 is for example a laser scanning unit. The light exposure section 28 exposes the charged surface of the image bearing member 1 to light to form an electrostatic latent image on the surface of the image bearing member 1. More specifically, the light exposure section 28 emits laser light based on image data input from a higher-level device, such as a computer, onto the surface of the image bearing member 1, which is uniformly charged by the charging section 27. Through the above, an electrostatic latent image based on the image data is formed on the surface of the image bearing member 1.

As already described above, the development section 29 develops the electrostatic latent image into a toner image. More specifically, the development section 29 supplies toner onto the surface of the image bearing member 1 on which the electrostatic latent image has been formed to form a toner image based on the image data. The toner image that is formed subsequently undergoes primary transfer onto the intermediate transfer belt 20. The toner has a positive charging polarity.

The development section 29 can develop the electrostatic latent image into a toner image while in contact with the image bearing member 1. That is, the image forming apparatus 6 according to the third embodiment can adopt a so-called contact development process. In the image forming apparatus 6 that adopts the contact development process, typically, the development roller and the image bearing member 1 are in contact with one another during development, and therefore a toner-component matter or a non-toner-component matter is likely to remain on and adhere to the surface of the image bearing member 1. It is thought that the matter adhering to the surface of the image bearing member 1 absorbs moisture and prevents the electrostatic latent image formed on the surface of the image bearing member 1 from being maintained in a stable manner. The image forming apparatus 6 according to the third embodiment tends to restrict hole injection to the photosensitive

layer of the photosensitive member 1. It is thought that the electrostatic latent image formed on the surface of the photosensitive member is therefore maintained in a stable manner. The image forming apparatus 6 according to the 5 third embodiment can therefore form images while reducing occurrence of black spots in a high temperature and humidity environment even through the contact development process.

The development section 29 can clean the surface of the 10 image bearing member 1. That is, the development section 29 can remove a residual matter from the surface of the image bearing member 1. The residual matter can prevent the electrostatic latent image from being maintained in a stable manner. As a result of the development section 29 15 cleaning the surface of the image bearing member 1 to remove the residual matter, therefore, the image forming apparatus 6 according to the third embodiment can form images while further reducing occurrence of black spots in a high temperature and humidity environment.

In order that the development section 29 efficiently cleans the surface of the image bearing member 1, the following 20 conditions (1) and (2) are preferably satisfied. Condition (1): A contact development process is employed, and rotation speed of the image bearing member and a 25 rotation speed of the development roller are different. Condition (2): A difference between a surface potential of the image bearing member 1 and a potential of the development bias satisfies relation (2-1) and relation (2-2) shown below.

$$0 (V) < \text{Potential } (V) \text{ of development bias} < \text{Surface potential } (V) \text{ of non-exposed region of image bearing member} \quad \text{Relation (2-1)}$$

$$\text{Potential } (V) \text{ of development bias} > \text{Surface potential } (V) \text{ of exposed region of image bearing member} \quad \text{Relation (2-2)}$$

In the relation (2-1), the surface potential of a non-exposed region of the image bearing member 1 refers to a surface potential of a region of the image bearing member 1 that has 40 not been exposed to light by the light exposure section 28. In the relation (2-2), the surface potential of an exposed region of the image bearing member 1 refers to a surface potential of a region of the image bearing member 1 that has been exposed to light by the light exposure section 28. Note 45 that the surface potential of the non-exposed region of the image bearing member 1 and the surface potential of the exposed region of the image bearing member 1 are measured after toner image transfer from the image bearing member 1 to the transfer target by the transfer section 26 and before 50 charging of the surface of the image bearing member 1 by the charging section 27 for the next rotation.

When the condition (1) is satisfied, that is, in a configuration in which the contact development process is adopted, and the rotation speed of the image bearing member 1 and 55 the rotation speed of the development roller are different, the surface of the image bearing member 1 is in contact with the development roller, and a residual matter on the surface of the image bearing member 1 is removed by rubbing against the development roller.

60 Preferably, the rotation speed of the image bearing member 1 is at least 120 mm/second and no greater than 350 mm/second. Preferably, the rotation speed of the development roller is at least 133 mm/second and no greater than 700 mm/second. Preferably, a ratio between the rotation speed  $V_P$  of the image bearing member 1 and the rotation speed  $V_D$  of the development roller satisfies relation (1-1) 65 shown below. The ratio being not equal to 1 means that the

## 21

rotation speed of the image bearing member 1 and the rotation speed of the development roller are different.

$$0.5 \leq V_P/V_D \leq 0.8$$

Relation (1-1)

The following describes the condition (2) taking, as an example, a configuration in which the toner has a positive charging polarity, and a reversal development process is adopted. When the condition (2) is satisfied, that is, in a configuration in which the potential of the development bias is different from the surface potential of the image bearing member 1, the surface potential (charge potential) of the image bearing member 1 and the potential of the development bias satisfy the relation (2-1) with respect to the non-exposed region. Accordingly, an electrostatic repulsion between remaining toner (hereinafter, may be referred to as residual toner) and the non-exposed region of the image bearing member 1 is greater than an electrostatic repulsion between the residual toner and the development roller. As a result, the residual toner moves from the surface of the image bearing member 1 to the development roller to be collected. The toner tends not to adhere to the non-exposed region of the image bearing member 1.

When the condition (2) is satisfied, that is, in a configuration in which the potential of the development bias is different from the surface potential of the image bearing member 1, the surface potential (sensitivity potential) of the image bearing member 1 and the potential of the development bias satisfy the relation (2-2) with respect to the exposed region. Accordingly, an electrostatic repulsion between the residual toner and the exposed region of the image bearing member 1 is smaller than an electrostatic repulsion between the residual toner and the development roller. As a result, the residual toner on the surface of the image bearing member 1 is maintained on the surface of the image bearing member 1. The toner adheres to the exposed region of the image bearing member 1.

The potential of the development bias is for example at least +250 V and no greater than +400 V. The charge potential of the image bearing member 1 is for example at least +450 V and no greater than +900 V. The sensitivity potential of the image bearing member 1 is for example at least +50 V and no greater than +200 V. The difference between the potential of the development bias and the charge potential of the image bearing member 1 is for example at least +150 V and no greater than +300 V. The difference between the potential of the development bias and the sensitivity potential of the image bearing member 1 is for example at least +100 V and no greater than +700 V. A potential difference herein refers to an absolute value of the difference. Such a potential difference can for example be established under conditions of a potential of the development bias of +330 V, a charge potential of the image bearing member 1 of +600 V, and a sensitivity potential of the image bearing member 1 of +100 V.

The intermediate transfer belt 20 is an endless circulating belt. The intermediate transfer belt 20 is wrapped against a drive roller 30, a driven roller 31, a backup roller 32, and the plurality of primary transfer rollers 33. The intermediate transfer belt 20 is located such that the surface of each of the image bearing members 1 is in contact with the circumferential surface of the intermediate transfer belt 20.

Furthermore, the intermediate transfer belt 20 is pressed against the image bearing members 1 by the primary transfer rollers 33. The endless intermediate transfer belt 20 is driven by the drive roller 30 to circulate while in a pressed state in an arrow direction (i.e., clockwise). The drive roller 30 is rotationally driven by a drive source, such as a stepping

## 22

motor, and imparts driving force that causes circulation of the endless intermediate transfer belt 20. The driven roller 31, the backup roller 32, and the primary transfer rollers 33 and passively rotate in accompaniment to circulation of the endless intermediate transfer belt 20 by the drive roller 30. The driven roller 31, the backup roller 32, and the primary transfer rollers 33 support the intermediate transfer belt 20.

The primary transfer rollers 33 are disposed opposite to the image bearing members 1 in one-to-one correspondence.

- 10 Each of the primary transfer rollers 33 transfers a toner image onto the intermediate transfer belt 20 from a corresponding one of the image bearing members 1. More specifically, the primary transfer rollers 33 each apply a primary transfer bias (more specifically, a bias of opposite polarity to toner charging polarity) to the intermediate transfer belt 20. As a result, toner images formed on the respective photosensitive members 1 are transferred (primary transfer) in order onto the circulating intermediate transfer belt 20. Each of the toner images is transferred onto the intermediate transfer belt 20 between the corresponding photosensitive member 1 and primary transfer roller 33.

The secondary transfer roller 21 applies a secondary transfer bias (more specifically, a bias of opposite polarity to the toner images) to paper P. As a result, the toner images that have undergone primary transfer onto the intermediate transfer belt 20 are transferred onto the paper P between the secondary transfer roller 21 and the backup roller 32. Through the above, an unfixed toner image is transferred onto the paper P.

- 25 30 The fixing section 10 fixes the unfixed toner image that has been transferred onto the paper P by the image forming section 9. The fixing section 10 includes a heating roller 34 and a pressure roller 35. The heating roller 34 is heated by a conductive heating element. The pressure roller 35 is located opposite to the heating roller 34 and has a circumferential surface that is pressed against a circumferential surface of the heating roller 34.

A transfer image that has been transferred onto paper P by the secondary transfer roller 21 in the image forming section 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9

process. Note that elements in FIG. 3 that correspond to elements in FIG. 2 are labelled using the same reference signs and redundant description is omitted.

As illustrated in FIG. 3, a transfer belt 40 is an endless circulating belt. The transfer belt 40 is wrapped against the drive roller 30, the driven roller 31, the backup roller 32, and the plurality of transfer rollers 41. The transfer belt 40 is located such that the surface of each of the image bearing members 1 is in contact with a surface (contact surface) of the transfer belt 40. The transfer rollers 41 are disposed opposite to the image bearing members 1 in one-to-one correspondence. The transfer belt 40 is pressed against the image bearing members 1 by the transfer rollers 41. The endless transfer belt 40 is driven by the plurality of rollers 30, 31, 32, and 41 to circulate while in a pressed state. The drive roller 30 is rotationally driven by a drive source, such as a stepping motor, and imparts driving force that causes circulation of the endless transfer belt 40. The driven roller 31, the backup roller 32, and the transfer rollers 41 are freely rotatable. The driven roller 31, the backup roller 32, and the transfer rollers 41 passively rotate in accompaniment to circulation of the endless transfer belt 40 by the drive roller 30. These rollers 31, 32, and 41 support the transfer belt 40 while also passively rotating. The paper P fed from the pair of registration rollers 17 is placed on the transfer belt 40 by a placement roller 42. The paper P placed on the transfer belt 40 passes between the image bearing members 1 and the transfer rollers 41 as the transfer belt 40 circulates.

The transfer section transfers toner images from the respective image bearing members 1 to the paper P as each of the image bearing members 1 comes in contact with the paper P. More specifically, each of the transfer rollers 41 applies a transfer bias (more specifically, a bias of opposite polarity to toner charging polarity) to the paper P placed on the transfer belt 40. As a result, a toner image formed on each of the photosensitive members 1 is transferred onto the paper P as the paper P passes between the photosensitive member 1 and the corresponding transfer roller 41. The transfer belt 40 is driven by the drive roller 30 to circulate in an arrow direction (i.e., clockwise). As the transfer belt 40 circulates, the paper P placed on the transfer belt 40 passes between the image bearing members 1 and the corresponding transfer rollers 41 in order. As the paper P passes between the image bearing members 1 and the corresponding transfer rollers 41, toner images of corresponding colors formed on the respective image bearing members 1 are transferred onto the paper P in order such that the toner images are superimposed on one another. Thereafter, the image bearing members 1 continue to rotate and a next process is performed. Through the above, description has been provided with reference to FIG. 3 for the image forming apparatus according to the alternative form of the third embodiment in which the direct transfer process is adopted.

As described with reference to FIGS. 2 and 3, the image forming apparatus 6 according to the third embodiment includes the photosensitive members 1 according to the first embodiment as image bearing members. The photosensitive members 1 have excellent sensitivity and can reduce occurrence of black spots in a high temperature and humidity environment. Including such photosensitive members 1 as image bearing members, the image forming apparatus 6 according to the third embodiment can form images while reducing occurrence of black spots in a high temperature and humidity environment with the photosensitive members 1 having excellent sensitivity.

#### Fourth Embodiment: Process Cartridge

5 The fourth embodiment of the present disclosure relates to a process cartridge. The process cartridge according to the fourth embodiment for example has a unitized configuration including the photosensitive member **1** of the first embodiment. The process cartridge may be designed to be freely attachable to and detachable from the image forming apparatus **6** according to the third embodiment. The process cartridge for example adopts a unitized configuration including, in addition to the photosensitive member **1**, one or more selected from the group consisting of the elements described for the third embodiment (more specifically, the charging section **27**, the light exposure section **28**, the development section **29**, the transfer section **26**, the cleaning section, and 10 the static eliminator).  
15

Through the above, the process cartridge according to the fourth embodiment has been described. The process cartridge according to the fourth embodiment includes the photosensitive member 1 according to the first embodiment.

20 The photosensitive member 1 according to the first embodiment has excellent sensitivity and can reduce occurrence of black spots in a high temperature and humidity environment. The process cartridge according to the fourth embodiment therefore provides excellent sensitivity and can form images while reducing occurrence of black spots in a high temperature and humidity environment. Furthermore, a process cartridge such as described above is easy to handle and can therefore be easily and quickly replaced, together with the image bearing member 1, when sensitivity characteristics or the like of the image bearing member 1 deteriorate.

## Examples

The following provides more specific description of the present disclosure through use of Examples. However, the present disclosure is not in any sense limited by the scope of the Examples.

## [1. Photosensitive Member Materials]

[1. Photosensitive Member Materials] A charge generating material, hole transport materials, electron transport materials, and a binder resin described below were prepared as materials for forming photosensitive layers of photosensitive members.

A compound (CGM-1X) was prepared as the charge generating material. The compound (CGM-1X) was metal-free phthalocyanine represented by the chemical formula (CGM-1) mentioned for the first embodiment. Furthermore, the compound (CGM-1X) had an X-form crystalline structure.

The compounds (HTM-1) to (HTM-6) were prepared as the hole transport materials. The compounds (HTM-1) to (HTM-6) have been described for the first embodiment.

The compounds (ETM-1) to (ETM-3) were prepared as the electron transport materials. The compounds (ETM-1) to (ETM-3) have been described in the first embodiment.



25

-continued



(ETM-5)



(ETM-6) 15



(ETM-7)

26

Next, a photosensitive layer formation step was performed. First, an application liquid was prepared. More specifically, 5 parts by mass of the compound (CGM-1X) as the charge generating material, 60 parts by mass of the compound (HTM-3) as the hole transport material, 35 parts by mass of the compound (ETM-1) as the electron transport material, 90 parts by mass of the polycarbonate resin (Za) as the binder resin, and 800 parts by mass of tetrahydrofuran as a solvent were added into a vessel. The vessel contents were mixed for 50 hours using a ball mill so that the materials were dispersed to give an application liquid.

Next, the application liquid was applied by dip coating onto the conductive substrate obtained through the oxide film formation step to form a film of the application liquid on the conductive substrate. More specifically, the conductive substrate was immersed in the application liquid. Next, the conductive substrate was drawn out of the application liquid. Through the above, the application liquid was applied onto the conductive substrate.

Next, the conductive substrate having a film of the application liquid was dried by hot air at 100° C. for 40 minutes. Thus, the solvent (tetrahydrofuran) was removed from the application liquid. As a result, a photosensitive layer was formed on the conductive substrate. Through the above, the photosensitive member (A-1) was obtained.

(2-2. Production of Photosensitive Members (A-2) to (A-18) and members (B-1) to (B-4) and (B-6) to (B-13))

The photosensitive members (A-2) to (A-18) and members (B-1) to (B-4) and (B-6) to (B-13) were produced in the same manner as in the production of the photosensitive member (A-1) except for the following changes.

Conditions for formation of the oxide film of the conductive substrate in the production of the photosensitive member (A-1) were changed. More specifically, the water temperature of 70° C., the water immersion time of 60 seconds, and the heating temperature 120° C. were changed to each water temperature, each water immersion time, and each heating temperature shown in Tables 1 and 2.

40 The compound (ETM-1) as the electron transport material and the compound (HTM-1) as the hole transport material that were used for preparation of the application liquid in the production of the photosensitive member (A-1) were changed to each electron transport material and each hole transport material shown in Tables 1 and 2.

[3. Measurement Methods]

(3-1. Measurement of Reduction Potential of Electron Transport Material)

The reduction potential of each electron transport material was determined by performing cyclic voltammetry under the following conditions.

Working electrode: glassy carbon

Counter electrode: platinum

Reference electrode: silver/silver nitrate (0.1 mol/L, a solution of AgNO<sub>3</sub> in acetonitrile)

Sample solution electrolyte: tetra-n-butylammonium perchlorate (0.1 mol)

Measurement target: electron transport material (0.001 mol)

Solvent: dichloromethane (1 L)

60 (3-2. Measurement of Leakage Onset Voltage of Photosensitive Member)

The leakage onset voltage of each photosensitive member was measured using a pressure-resistant tester (testing instrument fabricated by KYOCERA Document Solutions Inc.) under the following conditions.

Temperature: 30° C.

Relative humidity: 80%

A polycarbonate resin (Za) was prepared as the binder resin. The polycarbonate resin (Za) was the polycarbonate resin represented by the chemical formula (Z) described for the first embodiment. Furthermore, the viscosity average molecular weight of the polycarbonate resin (Za) was 40,000.

#### [2. Photosensitive Member Production]

Photosensitive members (A-1) to (A-16) and photosensitive members (B-1) to (B-4) and (B-6) to (B-13) were produced using the thus prepared materials for forming the photosensitive layers of the photosensitive members.

#### (2-1. Production of Photosensitive Member (A-1))

First, a conductive substrate was prepared. The conductive substrate was an aluminum conductive substrate having a diameter of 160 mm, a length of 365 mm, and a thickness of 2 mm. The conductive substrate was immersed in ionized alkaline water for 60 seconds, and subsequently an oxide film formation step was performed. The conductive substrate was immersed in water, taken out of the water, and heated to form an aluminum oxide film on a surface of the conductive substrate. The volume resistivity of the water was  $2.5 \times 10^6 \Omega \cdot \text{cm}$ . The temperature of the water was 80° C. The conductive substrate was immersed in the water for 30 seconds. The heating was performed using an oven at a heating temperature of 120° C. for 10 minutes at ambient atmosphere.

## (3-3. Proportion R of Oxygen Atoms Present in Surface of Conductive Substrate)

First, the surface of each conductive substrate was measured by energy dispersive X-ray spectroscopy (EDX) using an energy dispersive X-ray spectrometer ("JSM-6380LV", product of JEOL Ltd.). Measurement conditions were an accelerating voltage of 5 keV, an X-ray irradiation area of  $400 \mu\text{m}^2$ , and a measurement depth of 10 nm. Thus, the oxygen atom concentration ( $A_O$ , unit: atomic %) and the aluminum atom concentration ( $A_{Al}$ , unit: atomic %) in the surface of the conductive substrate were measured. Based on the oxygen atom concentration and the aluminum atom concentration that were measured, the proportion R of oxygen atoms present in the surface of the conductive substrate was calculated in accordance with equation (1) shown below. Tables 1 and 2 show the thus calculated proportion R of oxygen atoms.

$$R = [A_O / (A_O + A_{Al})] \times 100 \quad \text{Equation (1)}$$

## (3-4. Measurement of Oxide Film Thickness)

The oxide film thickness was measured using a reflective/transmissive thin film thickness measuring device ("NANO-CALC-VIS", product of Tokyo Instruments, Inc.). Tables 1 and 2 show the thus measured oxide film thickness.

## [4. Evaluation Methods]

## (4-1. Image Evaluation (Black Spots))

A printer (dry-type electrophotographic printer including a semiconductor laser, "FS-1300D", product of KYOCERA Document Solutions Inc.) was used as an evaluation apparatus. The evaluation apparatus included a charging roller as a charging section. The charging section had a positive charging polarity. The evaluation apparatus included a direct-transfer type transfer section (transfer roller). The evaluation apparatus included a development section having a photosensitive member cleaning function. "KYOCERA Document Solutions-brand paper VM-A4 (A4 size)", product of KYOCERA Document Solutions Inc. was used as paper for evaluations. "Non-magnetic one-component toner", product of KYOCERA Document Solutions Inc. was

used as a toner for the evaluations. Measurements for the evaluations were carried out in a high temperature and humidity environment (temperature:  $32.5^\circ \text{C}$ , relative humidity: 80%). With respect to each of the photosensitive members, the photosensitive member was mounted in the evaluation apparatus. An image was formed under a condition of a linear velocity of 168 mm/second. In order to stabilize the operation of the photosensitive member in the evaluation apparatus, an alphabetical image was printed on 1,000 sheets of the paper. Subsequently, an image D was printed on a sheet and used as an evaluation sample for black spot evaluation. The image D was an entirely white image. The thus obtained evaluation sample was visually observed to determine presence of black spots. Based on the observation result, image evaluation was performed in terms of black spots as an image defect in accordance with the following evaluation standard.

## (Evaluation Standard of Image Evaluation in terms of Black Spots)

G (Good): five or less black spots

P (Poor): more than 5 black spots

## (4-2. Measurement of Sensitivity Potential of Photosensitive Member)

The sensitivity potential of each photosensitive member was measured using a drum sensitivity test device (Gentec Inc.) under environmental conditions of a temperature of  $10^\circ \text{C}$ . and a relative humidity of 20%. The surface of the photosensitive member was charged to a surface potential of  $+600 \text{ V}$ . Thereafter, the surface of the photosensitive member was exposed to monochromatic light (light exposure wavelength: 780 nm) at a light exposure amount of  $0.26 \mu\text{J}/\text{cm}^2$ . A surface potential ( $V_L$ ) of an exposed region of the photosensitive member was measured 50 milliseconds after exposure to the light. Sensitivity of the photosensitive member was evaluated in accordance with the following standard.

G (Good): a surface potential ( $V_L$ ) of no greater than  $+130 \text{ V}$

P (Poor): a surface potential ( $V_L$ ) of greater than  $+130 \text{ V}$

TABLE 1

| Example    | Photo-sensitive member No. | Conductive substrate              |                          |                                     |            |       | Proportion of oxygen atoms (%) | Oxide film thickness ( $\mu\text{m}$ ) | Type | Photo-sensitive layer | Electron transport | Photo-sensitive member |  |  |  |  |  |  |
|------------|----------------------------|-----------------------------------|--------------------------|-------------------------------------|------------|-------|--------------------------------|----------------------------------------|------|-----------------------|--------------------|------------------------|--|--|--|--|--|--|
|            |                            | Oxide film formation step         |                          |                                     | Proportion | Oxide |                                |                                        |      |                       |                    |                        |  |  |  |  |  |  |
|            |                            | Water temp. ( $^\circ \text{C}$ ) | Immersion time (seconds) | Heating temp. ( $^\circ \text{C}$ ) |            |       |                                |                                        |      |                       |                    |                        |  |  |  |  |  |  |
| Example 1  | A-1                        | 70                                | 60                       | 120                                 | 22         | 0.16  | ETM-1                          | -0.88                                  | 5.00 |                       |                    |                        |  |  |  |  |  |  |
| Example 2  | A-2                        | 70                                | 90                       | 120                                 | 26         | 0.20  | ETM-1                          | -0.88                                  | 5.10 |                       |                    |                        |  |  |  |  |  |  |
| Example 3  | A-3                        | 80                                | 15                       | 120                                 | 21         | 0.16  | ETM-1                          | -0.88                                  | 5.20 |                       |                    |                        |  |  |  |  |  |  |
| Example 4  | A-4                        | 80                                | 30                       | 120                                 | 26         | 0.20  | ETM-1                          | -0.88                                  | 5.20 |                       |                    |                        |  |  |  |  |  |  |
| Example 5  | A-5                        | 80                                | 60                       | 120                                 | 30         | 0.24  | ETM-1                          | -0.88                                  | 5.50 |                       |                    |                        |  |  |  |  |  |  |
| Example 6  | A-6                        | 80                                | 90                       | 120                                 | 38         | 0.30  | ETM-1                          | -0.88                                  | 5.60 |                       |                    |                        |  |  |  |  |  |  |
| Example 7  | A-7                        | 80                                | 15                       | 110                                 | 21         | 0.16  | ETM-1                          | -0.88                                  | 5.20 |                       |                    |                        |  |  |  |  |  |  |
| Example 8  | A-8                        | 80                                | 15                       | 120                                 | 21         | 0.16  | ETM-1                          | -0.88                                  | 5.10 |                       |                    |                        |  |  |  |  |  |  |
| Example 9  | A-9                        | 80                                | 15                       | 150                                 | 21         | 0.16  | ETM-1                          | -0.88                                  | 5.20 |                       |                    |                        |  |  |  |  |  |  |
| Example 10 | A-10                       | 95                                | 5                        | 120                                 | 20         | 0.15  | ETM-1                          | -0.88                                  | 5.10 |                       |                    |                        |  |  |  |  |  |  |
| Example 11 | A-11                       | 95                                | 15                       | 120                                 | 28         | 0.21  | ETM-1                          | -0.88                                  | 5.30 |                       |                    |                        |  |  |  |  |  |  |
| Example 12 | A-12                       | 95                                | 30                       | 120                                 | 34         | 0.28  | ETM-1                          | -0.88                                  | 5.50 |                       |                    |                        |  |  |  |  |  |  |
| Example 13 | A-13                       | 95                                | 60                       | 120                                 | 40         | 0.32  | ETM-1                          | -0.88                                  | 5.60 |                       |                    |                        |  |  |  |  |  |  |
| Example 14 | A-14                       | 95                                | 90                       | 120                                 | 46         | 0.35  | ETM-1                          | -0.88                                  | 5.80 |                       |                    |                        |  |  |  |  |  |  |
| Example 15 | A-15                       | 80                                | 15                       | 120                                 | 21         | 0.16  | ETM-2                          | -0.70                                  | 5.40 |                       |                    |                        |  |  |  |  |  |  |
| Example 16 | A-16                       | 80                                | 15                       | 120                                 | 21         | 0.16  | ETM-3                          | -0.66                                  | 5.60 |                       |                    |                        |  |  |  |  |  |  |
| Example 17 | A-17                       | 95                                | 90                       | 120                                 | 34         | 0.28  | ETM-2                          | -0.70                                  | 5.80 |                       |                    |                        |  |  |  |  |  |  |
| Example 18 | A-18                       | 95                                | 90                       | 120                                 | 34         | 0.28  | ETM-3                          | -0.66                                  | 6.20 |                       |                    |                        |  |  |  |  |  |  |

TABLE 2

| Photo-sensitive<br>member<br>No. | Conductive substrate     |                             |                         |                    |          | Proportion<br>of oxygen<br>atoms (%) | Oxide<br>filmthick-<br>ness (μm) | Type  | Reduction<br>potential (V) | onset volt-<br>age (kV) |  |  |  |  |  |
|----------------------------------|--------------------------|-----------------------------|-------------------------|--------------------|----------|--------------------------------------|----------------------------------|-------|----------------------------|-------------------------|--|--|--|--|--|
|                                  | Oxide filmformation step |                             |                         | Electron transport | material |                                      |                                  |       |                            |                         |  |  |  |  |  |
|                                  | Water<br>temp. (° C.)    | Immersion<br>time (seconds) | Heating<br>temp. (° C.) |                    |          |                                      |                                  |       |                            |                         |  |  |  |  |  |
| Comparative Example 1            | B-1                      | —                           | —                       | —                  | 1        | 0                                    | ETM-1                            | -0.88 | 4.50                       |                         |  |  |  |  |  |
| Comparative Example 2            | B-2                      | 70                          | 5                       | 120                | 3        | 0                                    | ETM-1                            | -0.88 | 4.70                       |                         |  |  |  |  |  |
| Comparative Example 3            | B-3                      | 70                          | 15                      | 120                | 5        | 0                                    | ETM-1                            | -0.88 | 4.80                       |                         |  |  |  |  |  |
| Comparative Example 4            | B-4                      | 70                          | 30                      | 120                | 8        | 0.06                                 | ETM-1                            | -0.88 | 4.80                       |                         |  |  |  |  |  |
| Comparative Example 6            | B-6                      | 80                          | 15                      | 120                | 21       | 0.15                                 | ETM-4                            | -0.96 | 4.00                       |                         |  |  |  |  |  |
| Comparative Example 7            | B-7                      | 80                          | 15                      | 120                | 21       | 0.15                                 | ETM-5                            | -0.93 | 4.40                       |                         |  |  |  |  |  |
| Comparative Example 8            | B-8                      | 80                          | 15                      | 120                | 21       | 0.15                                 | ETM-6                            | -0.93 | 4.50                       |                         |  |  |  |  |  |
| Comparative Example 9            | B-9                      | 80                          | 15                      | 120                | 21       | 0.15                                 | ETM-7                            | -0.55 | 6.00                       |                         |  |  |  |  |  |
| Comparative Example 10           | B-10                     | 95                          | 90                      | 120                | 46       | 0.35                                 | ETM-4                            | -0.96 | 4.50                       |                         |  |  |  |  |  |
| Comparative Example 11           | B-11                     | 95                          | 90                      | 120                | 46       | 0.35                                 | ETM-5                            | -0.93 | 4.80                       |                         |  |  |  |  |  |
| Comparative Example 12           | B-12                     | 95                          | 90                      | 120                | 46       | 0.35                                 | ETM-6                            | -0.93 | 4.80                       |                         |  |  |  |  |  |
| Comparative Example 13           | B-13                     | 95                          | 90                      | 120                | 46       | 0.35                                 | ETM-7                            | -0.55 | 6.40                       |                         |  |  |  |  |  |
| Comparative Example 14           | B-14                     | 80                          | 60                      | 120                | 30       | 0.24                                 | —                                | —     | 4.50                       |                         |  |  |  |  |  |

As shown in Table 1, the photosensitive layer of each of the photosensitive members (A-1) to (A-18) included any of the electron transport materials (ETM-1) to (ETM-3). The reduction potential of the electron transport materials (ETM-1) to (ETM-3) was within a range of from -0.88 V to -0.66 V versus the reference electrode (Ag/Ag<sup>+</sup>). The leak onset voltage of the photosensitive members (A-1) to (A-18) in the high temperature and humidity environment was within a range of from 5.00 kV to 6.20 kV. The photosensitive members (A-1) to (A-18) each had an aluminum oxide film.

As shown in Table 2, the leakage onset voltage of the photosensitive members (B-1) to (B-4) was within a range of from 4.50 kV to 4.90 kV. The photosensitive layer of each of the photosensitive members (B-6) to (B-13) contained any of the electron transport materials (ETM-4) to (ETM-7). The reduction potential of the electron transport materials (ETM-4) to (ETM-7) was within a range of from -0.96 V to -0.93 V or was -0.55 V versus the reference electrode (Ag/Ag<sup>+</sup>). The leakage onset voltage of the photosensitive members (B-6) to (B-8) and the photosensitive members (B-10) to (B-12) was within a range of from 4.00 kV to 4.80 kV.

TABLE 3-continued

| 35 | Photo-sensitive<br>member<br>No. | Image defect        |                 | Electrical properties<br>(sensitivity) |                 |
|----|----------------------------------|---------------------|-----------------|----------------------------------------|-----------------|
|    |                                  | Black spot<br>count | Evalu-<br>ation | Sensitiv-<br>ity<br>potential (V)      | Evalu-<br>ation |
| 40 | Example 6                        | A-6                 | 2               | G                                      | +122            |
|    | Example 7                        | A-7                 | 4               | G                                      | +118            |
|    | Example 8                        | A-8                 | 5               | G                                      | +119            |
|    | Example 9                        | A-9                 | 4               | G                                      | +117            |
|    | Example 10                       | A-10                | 3               | G                                      | +122            |
|    | Example 11                       | A-11                | 4               | G                                      | +119            |
| 45 | Example 12                       | A-12                | 3               | G                                      | +123            |
|    | Example 13                       | A-13                | 2               | G                                      | +117            |
|    | Example 14                       | A-14                | 1               | G                                      | +120            |
|    | Example 15                       | A-15                | 3               | G                                      | +118            |
|    | Example 16                       | A-16                | 2               | G                                      | +119            |
| 50 | Example 17                       | A-17                | 2               | G                                      | +117            |
|    | Example 18                       | A-18                | 1               | G                                      | +118            |

TABLE 4

| 55 | Photo-sensitive<br>member<br>No. | Image defect        |                 | Electrical properties<br>(sensitivity) |                 |
|----|----------------------------------|---------------------|-----------------|----------------------------------------|-----------------|
|    |                                  | Black spot<br>count | Evalu-<br>ation | Sensitiv-<br>ity<br>potential (V)      | Evalu-<br>ation |
| 60 | Comparative Example 1            | B-1                 | 22              | P                                      | +119            |
|    | Comparative Example 2            | B-2                 | 15              | P                                      | +117            |
|    | Comparative Example 3            | B-3                 | 10              | P                                      | +120            |
| 65 | Comparative Example 4            | B-4                 | 9               | P                                      | +118            |

TABLE 3

| Photo-sensitive<br>member<br>No. | Image defect        |                 | Electrical properties<br>(sensitivity) |                 |
|----------------------------------|---------------------|-----------------|----------------------------------------|-----------------|
|                                  | Black spot<br>count | Evalu-<br>ation | Sensitiv-<br>ity<br>potential (V)      | Evalu-<br>ation |
| Example 1                        | A-1                 | 4               | G                                      | +119            |
| Example 2                        | A-2                 | 3               | G                                      | +119            |
| Example 3                        | A-3                 | 3               | G                                      | +117            |
| Example 4                        | A-4                 | 3               | G                                      | +118            |
| Example 5                        | A-5                 | 3               | G                                      | +121            |

TABLE 4-continued

| Photo-sensitive member No. | Image defect | Electrical properties (sensitivity) |            |                           | Evaluation |
|----------------------------|--------------|-------------------------------------|------------|---------------------------|------------|
|                            |              | Black spot count                    | Evaluation | Sensitivity potential (V) |            |
| Comparative Example 6      | B-6          | 31                                  | P          | +118                      | G          |
| Comparative Example 7      | B-7          | 25                                  | P          | +119                      | G          |
| Comparative Example 8      | B-8          | 24                                  | P          | +117                      | G          |
| Comparative Example 9      | B-9          | 1                                   | G          | +178                      | P          |
| Comparative Example 10     | B-10         | 24                                  | P          | +122                      | G          |
| Comparative Example 11     | B-11         | 19                                  | P          | +117                      | G          |
| Comparative Example 12     | B-12         | 18                                  | P          | +119                      | G          |
| Comparative Example 13     | B-13         | 1                                   | G          | +178                      | P          |

As shown in Table 3, both the result of the image evaluation and the result of the sensitivity evaluation of each of the photosensitive members (A-1) to (A-18) were G (Good). As shown in Table 4, the result of the image evaluation or the result of the sensitivity evaluation of each of the photosensitive members (B-1) to (B-4) and (B-6) to (B-13) was P (Poor). More specifically, the result of the image evaluation of each of the photosensitive members (B-1) to (B-4) and (B-6) to (B-8) and the photosensitive members (B-10) to (B-12) was P (Poor). The result of the sensitivity evaluation of each of the photosensitive member (B-9) and the photosensitive member (B-13) was P (Poor).

The evaluation results indicate that the photosensitive members (A-1) to (A-18) are superior to the photosensitive members (B-1) to (B-4) and (B-6) to (B-13) in sensitivity and capability of reducing occurrence of black spots in a high temperature and humidity environment.

What is claimed is:

1. A single-layer electrophotographic photosensitive member comprising a conductive substrate and a photosensitive layer disposed directly on the conductive substrate, wherein
  - the conductive substrate contains aluminum or an aluminum alloy,
  - a surface of the conductive substrate has a film of an oxide of the aluminum or a film of an oxide of the aluminum alloy,
  - the film of the oxide of the aluminum or the film of the oxide of the aluminum alloy has a thickness of at least 0.15  $\mu\text{m}$  and no greater than 0.35  $\mu\text{m}$ ,
  - the photosensitive layer contains a charge generating material and an electron transport material, the charge generating material is X-form metal-free phthalocyanine,
  - the electron transport material has a reduction potential of at least  $-0.88 \text{ V}$  and no greater than  $-0.66 \text{ V}$  versus a reference electrode ( $\text{Ag}/\text{Ag}^+$ ),
  - the single-layer electrophotographic photosensitive member has a leakage onset voltage of at least 5.0 kV in a high temperature and humidity environment at a temperature of  $30^\circ \text{C}$ . and a relative humidity of 80%, the leakage onset voltage being a voltage applied to the single-layer electrophotographic photosensitive member at which current leakage starts,

the electron transport material includes a compound represented by general formula (2) or general formula (3) shown below,



where in the general formulae (2) and (3),

$\text{R}^3$ ,  $\text{R}^4$ ,  $\text{R}^5$ ,  $\text{R}^6$ ,  $\text{R}^7$ , and  $\text{R}^8$  each represent, independently of one another, an alkyl group that may have a substituent selected from the group consisting of alkoxy groups and halogen atoms or an aryl group that may have a substituent selected from the group consisting of alkoxy groups and halogen atoms, and

a proportion R of oxygen atoms present in the film of an oxide of the aluminum or the film of an oxide of the aluminum alloy is at least 20% and no greater than 50%, the proportion R being calculated in accordance with equation (1) shown below,

$$R = [\text{A}_O / (\text{A}_O + \text{A}_{\text{Al}})] \times 100 \quad \text{Equation (1)}$$

where in the equation (1),

$\text{A}_O$  represents an oxygen atom concentration determined by measuring the film of an oxide of the aluminum or the film of an oxide of the aluminum alloy by energy dispersive X-ray spectroscopy, and

$\text{A}_{\text{Al}}$  represents an aluminum atom concentration determined by measuring the film of an oxide of the aluminum or the film of an oxide of the aluminum alloy by energy dispersive X-ray spectroscopy.

2. The single-layer electrophotographic photosensitive member according to claim 1, wherein

in the general formulae (2) and (3),

$\text{R}^3$ ,  $\text{R}^4$ ,  $\text{R}^5$ ,  $\text{R}^7$ , and  $\text{R}^8$  each represent, independently of one another, an alkyl group having a carbon number of at least 1 and no greater than 5, and

$\text{R}^6$  represents a phenyl group having a halogen atom.

3. The single-layer electrophotographic photosensitive member according to claim 1, wherein

the electron transport material includes a compound represented by chemical formula (ETM-2) or chemical formula (ETM-3) shown below

33



34

(ETM-2) 4. A process cartridge comprising the single-layer electrophotographic photosensitive member according to claim 1.

5 5. An image forming apparatus comprising:  
an image bearing member; and  
a charger configured to charge a surface of the image bearing member, wherein  
10 the charger has a positive charging polarity, and  
the image bearing member is the single-layer electrophotographic photosensitive member according to claim 1.

15 6. The image forming apparatus according to claim 5,  
further comprising  
a development section configured to develop an electrostatic latent image into a toner image while in contact  
20 with the image bearing member.

7. The image forming apparatus according to claim 6,  
wherein  
the development section cleans the surface of the image bearing member.

25 8. The image forming apparatus according to claim 5,  
wherein  
the charger is a charging roller.

\* \* \* \* \*